

1

3,445,205

## FUEL OIL COMPOSITION HAVING IMPROVED LOW TEMPERATURE PROPERTIES

Seymour H. Patinkin, Chicago, Ill., James H. Kirk, Dyer, Ind., and William L. Steinhoff, South Holland, Ill., assignors to Sinclair Research Inc., New York, N.Y., a corporation of Delaware

No Drawing. Filed Sept. 25, 1964, Ser. No. 399,334

Int. Cl. C10I 1/18

U.S. Cl. 44—62

3 Claims

### ABSTRACT OF THE DISCLOSURE

A fuel composition having improved low temperature properties is prepared by incorporating into a petroleum distillate fuel boiling having the gasoline range minor amounts of an acrylic acid ester polymer pour depressor and a petroleum microcrystalline wax having a melting point up to about 145° F. and derived from a Mid-Continent base crude oil. The fuel compositions of this invention have reduced pour point and improved low temperature pumpability.

This invention relates to distillate fuel oil compositions having improved pour point and pumpability characteristics at low temperatures. More particularly, the present invention is directed to haze-free distillate mineral fuel oils boiling above the gasoline range containing in combination small amounts of an acrylic acid ester polymer pour depressor and certain microcrystalline waxes derived from mixed base crude oils, often called Mid-Continent crudes.

In order to meet pour point specifications for petroleum distillate fuel oils such as heating oils, diesel fuels and the like it is frequently necessary to incorporate a pour depressor. Many materials are known pour depressors and among these a highly effective class is represented by a group of synthetic resins derived by the polymerization of esters of acrylic acid, including methacrylic esters. It is also known in the prior art that the effect of these acrylic acid ester polymer pour depressors can be aided or assisted by incorporating along with them a small amount of certain microcrystalline waxes. See, for instance U.S. Patent No. 2,917,375 to Charles N. Hudson wherein is disclosed that microcrystalline waxes derived from paraffinic base oils in conjunction with acrylate polymers are good pour depressants in fuel oils and eliminate hazy formation in the oils. Also demonstrated by the patentee is the fact that microcrystalline waxes obtained from mixed base crudes, on the other hand, when added to the same fuel oils in combination with the acrylate polymers caused the fuel to become hazy at moderate temperatures such as 40° F.

We have now discovered that certain microcrystalline waxes obtained from mixed base or Mid-Continent crude oils, are excellent pour depressant aids and pumpability aids for distillate fuels containing an acrylate pour depressor. In addition the use of the microcrystalline waxes of the invention does not cause an objectionable haze at reduced temperatures.

The microcrystalline waxes of the present invention are, as aforementioned, derived from mixed or Mid-Continent crude oils, and are characterized by a melting point of about 145° F. maximum, preferably below about 100° F. The microcrystalline waxes can be obtained from Mid-Continent petrolatums by eliminating the high melt portion of the petrolatums. For example, the microcrystalline waxes of the invention can be produced by partial crystallization of the parent petroatum, as for instance, by dissolving one part of the Mid-Continent microcrystalline wax into five (5) parts of hot 300° to 400° F. naphtha and collecting the high melting precipitate formed at room

2

temperature. The resulting solution is then solvent stripped to obtain the desired low melting microcrystalline wax.

Similarly, the microcrystalline waxes of the invention can be obtained by conventional solvent deoiling wherein petroatum is dissolved in methyl ethyl ketone or mixtures of methyl ethyl ketone and toluene or similar solvent systems and the high melt wax precipitate at reduced temperatures. The portion of petroatum which is soluble in the solvent at the temperature of crystallization is generally known as foots oil and is predominantly microcrystalline wax. Depending on the solvent deoiling conditions employed a single deoiling or a succession of solvent deoilings of the foots oil produced in each step may be used to obtain the microcrystalline wax of the invention.

15 The acrylic acid ester pour depressors to be used in the instant invention are known materials and include those available commercially as the Acryloids such as Acryloid 150 (a methacrylate ester polymer prepared from cetyl, lauryl and octyl alcohols with a molecular weight of about 10,000 to 15,000), Acryloid 710 (a methacrylate ester polymer prepared from lauryl and octyl alcohols with a molecular weight of about 10,000 to 20,000), and Acryloid 763 (a 40% by weight concentrate of acrylate in a hydrocarbon solvent having an API gravity of about 24.0 and a viscosity at 210° F. of about 3577 SUS). These resins are oil-soluble and include, for instance polymerized esters of alpha-methacrylic acid or acrylic acid and monohydric aliphatic saturated alcohols. The alcohols employed are generally those having at least 20 about 8 carbon atoms on the average and preferably about 12 to 24 or more carbon atoms per molecule. Typical pour depressors are polymers of dodecyl methacrylate, tetradecyl methacrylate, hexadecyl methacrylate, and octadecyl methacrylate. The polymers often have molecular weights of about 500 to 20,000. In commercial form, the pour depressors are available as a 40 weight percent concentrate in a high grade hydrocarbon solvent. These concentrates normally have API gravities of about 23 to 28, and a viscosity at 210° F. of about 2500 to 4000 SUS.

25 Improved pour point and pumpability of fuels at very low temperatures; e.g. from the cloud point of a fuel, which may be as high as +15° F. or higher, to -15° F. or lower, can be obtained by incorporating in the fuel small effective amounts, for instance at least about 0.001 volume percent, often about 0.003 volume percent to 30 0.1 volume percent (dry basis), preferably about 0.01 to 0.05 volume percent, of the acrylic type pour depressor, and at least about 0.1 volume percent up to about 35 1 volume percent, preferably about 0.2 to 0.5 volume percent, of the microcrystalline wax. Higher concentrations of either component can be used, but they are less desirable from an economic viewpoint and in most cases excellent pour depression and pumpability are obtained 40 within the above limits. The best additive combination 45 may differ from fuel to fuel since susceptibility to the additives may vary with fuel composition.

45 Compositions of the present invention can be produced by incorporating the microcrystalline wax in the mineral oil fraction either before or after the pour depressor is 50 added, or the depressor aid can be added to the pour depressor separately from the oil and then incorporated in the oil as a mixture with the pour depressor. Microcrystalline waxes generally are highly soluble in acrylic type pour depressors and, of course, both the waxes and 55 the acrylate pour depressor are highly soluble in mineral oils generally. Special conditions of temperature and pressure need not be observed in effecting solution of the additives in the oil. To form a solution of the acrylate pour depressor and the wax in the absence of the distillate fuel, it may be desirable to heat them to an elevated temperature, e.g. to about 125° F., to effect solution.

60 The hydrocarbon fuel oils which are improved in ac-

cordance with this invention are the normally liquid petroleum distillates boiling primarily above the gasoline range and include, for example, diesel fuels, heating oils, etc. These oils are usually petroleum middle distillates, which generally boil primarily in the range of about 250° to 750° F., and commonly have relatively high pour points, for instance, at least at -10° F. or higher. The oils can be in their relatively crude state or they can be treated in accordance with well-known commercial methods such as acid or caustic treatment, solvent refining, hydrotreating, etc. The fuel oils can contain straight run distillate fuel oils, catalytically or thermally cracked fuel oils or mixtures of straight run fuel oils, naphthas and the like with cracked distillate stocks. The cracked materials will frequently be about 15 to 70 volume percent of the fuel.

The following examples are included to further illustrate the present invention.

#### Example I

A petrolatum derived from a Mid-Continent crude oil and having a cone penetration at 77° F. of 62 was subjected to conventional solvent deoiling at 40-45° F. using a 50-50 mixture of toluene and methyl ethyl ketone. The ratio of solvent to petroleum employed was 4 to 1. The precipitated wax was filtered to provide a wax cake (52.7%) and foots oil (47.3%). The foots oil was designated CFO-IN.

#### Example II

The wax cake of Example I, 88 SUS at 210° F., 32 cone penetration at 77° F. was deoiled as in Example I employing a solvent to wax cake ratio of 3 to 1 and a temperature of 40-45° F. to provide after filtration a second pass wax (85%) and foots oil filtrate (15%). The foots oil was designated CFO-2N.

#### Example III

The wax of Example II, 17 cone penetration at 77° F., was deoiled as in Examples I and II but employing a 45-50° F. crystallization temperature to produce after filtration a third pass wax (90%), 45 cone penetration at 110° F., and foots oil filtrate (10%). The foots oil was designated CFO-3N.

#### Example IV

A 100 gram portion of a Mid-Continent petrolatum having an API gravity of 30.9° and a cone penetration at 77° F. of 61.0 was dissolved in 500 grams of naphtha by heating to 140-145° F. The solution was permitted to cool to 77° F. During the cooling the cloud point was determined to be 113.5° F. When the wax slurry was at the dewaxing temperature, a 20% by weight portion of Hyflo Super Cel (diatomaceous earth) was added to improve filterability and the slurry filtered at the dewaxing temperature on a Buchner funnel. The resulting microcrystalline wax was designated ECDH.

The inspections of the foots oil microcrystalline waxes CFO-IN, CFO-2N, CFO-3N and the microcrystalline wax ECDH prepared in Examples I to IV above are summarized in Table I below. An inspection of a Mid-Continent petroleum used for purposes of comparison in Examples to follow is also included as are other waxes identified in Table I.

TABLE I.—MICROCRYSTALLINE WAX INSPECTIONS

|                            | CFO-1N | CFO-2N | CFO-3N | CFO-CN <sup>1</sup> | CFO-CB <sup>2</sup> | CFO-2 <sup>3</sup> | ECDH  | Petrolatum A |
|----------------------------|--------|--------|--------|---------------------|---------------------|--------------------|-------|--------------|
| Melting Point, °F.         | <100   | <100   | <100   | <100                | <100                | 103                | 103   | 161          |
| Congealing Point, °F.      | 83     | 88     | 106    | 88                  | 106                 | 118                | 118   | 61           |
| Cone Penetration at 77° F. | 223    | 248    | 70     | 207                 | 171                 | 212                | 212   | 31.9         |
| Gravity, °API              | 30     | 31.3   | 32.8   | 30.2                | 31.8                | 30.2               | 30.2  | 590          |
| Flash, °F.                 | 600    | 575    | 545    | 588                 | 575                 | 575                | 575   | 650          |
| Fire, °F.                  | 650    | 645    | 625    | 640                 | 645                 | 650                | 650   | 7.4          |
| Percent Oil                | 9.8    | 8.1    | 3.6    | 8.6                 | 6.9                 | 10.0               | 10.0  | 98.0         |
| Viscosity at 210° F., SUS  | 113    | 101.4  | 88.5   | 107.2               | 100.4               | 100.4              | 100.4 | 98.0         |

<sup>1</sup> A microwax combination of at least 2 of CFO-1N, CFO-2N and CFO-3N.

<sup>2</sup> A microwax combination of a series of CFO-2N waxes.

<sup>3</sup> A second pass foots oil microcrystalline wax obtained according to Examples I and II but employing a different starting Mid-Continent petrolatum.

#### Example V

Samples of No. 2 fuel oils from different sources containing small concentrations of either Acryloid 763 alone, the microcrystalline waxes identified in Table I above as CFO-1N, CFO-2N and CFO-3N and a combination of both Acryloid 763 and the waxes were made up and the pour points, ASTM (D-97), of the samples determined. The No. 2 fuels utilized had the following inspections:

|                            | Fuel Oil A | Fuel Oil B |
|----------------------------|------------|------------|
| Composition:               |            |            |
| Water White Distillate     | 65         | 55         |
| Gas Oil                    | 30         | 30         |
| Light Cycle Oil            | 5          | 5          |
| Kerosene                   |            |            |
| Laboratory Tests:          |            |            |
| Gravity, °API              | 33.9       | 34.6       |
| Flash, °F. PM              | 150        | 136        |
| Viscosity at 100° F., c.s. | 2.813      | 2.548      |
| Cloud Point, °F.           | +2         | +4         |
| Pour Point, °F.            | -5         | -5         |
| Olefins, FIA, percent      | 0.2        | 0.2        |
| Aromatics, FIA, percent    | 30.1       | 33.2       |
| Sulfur, percent            | 0.34       | 0.39       |
| Bromine Number             | 4.0        | 7.7        |
| Distillation:              |            |            |
| IBP, °F.                   | 305        | 330        |
| 10%                        | 380        | 406        |
| 50%                        | 552        | 514        |
| 90%                        | 584        | 594        |
| E.P.                       | 618        | 632        |
| Recovery                   | 98         | 98         |

The pour point results are shown in Table II below:

TABLE II

| Additive, Vol. percent | Foots Oil | Fuel Oil A |       | Fuel Oil B |       |
|------------------------|-----------|------------|-------|------------|-------|
|                        |           | CFO-1N     | 21284 | 21377      | 21315 |
| 0.00                   | 0.0       | -5         | -5    | -5         | -10   |
| 0.00                   | 0.1       | -5         | 0     | -5         | -5    |
| 0.00                   | 0.2       | -5         | 0     | -5         | -10   |
| 0.00                   | 0.3       | -5         | -5    | -5         | -5    |
| 0.01                   | 0.0       | -5         | -5    | -5         | -10   |
| 0.03                   | 0.0       | -5         | -5    | -5         | -10   |
| 0.05                   | 0.0       | -5         | -10   | -10        | -10   |
| 0.01                   | 0.2       | -5         | -5    | -15        | -20   |
| 0.03                   | 0.2       | -10        | -15   | -15        | -20   |
| 0.05                   | 0.2       | -10        | -15   | -15        | -20   |
| 0.01                   | 0.3       | -10        | +5    | -15        | -10   |
| 0.03                   | 0.3       | -20        | -5    | -30        | -45   |
| 0.05                   | 0.3       | -25        | -30   | -35        | -30   |
| Foots Oil              |           |            |       |            |       |
| CFO-2N                 |           |            |       |            |       |
| 0.00                   | 0.1       | -5         | +5    | -5         | -5    |
| 0.00                   | 0.2       | -5         | 0     | -5         | -5    |
| 0.00                   | 0.3       | -5         | +5    | -5         | -5    |
| 0.01                   | 0.2       | -10        | -5    | -10        | -20   |
| 0.03                   | 0.2       | -10        | -20   | -20        | -25   |
| 0.05                   | 0.2       | -15        | -20   | -20        | -30   |
| 0.01                   | 0.3       | -10        | +5    | -10        | -15   |
| 0.03                   | 0.3       | -35        | 0     | -20        | -40   |
| 0.05                   | 0.3       | -30        | -5    | -30        | -40   |
| 0.00                   | 0.1       | -5         | +5    | -5         | -5    |
| 0.00                   | 0.2       | -5         | +5    | -5         | -10   |
| 0.00                   | 0.3       | -5         | +5    | -5         | -10   |
| 0.01                   | 0.2       | -30        | +10   | -10        | -15   |
| 0.03                   | 0.2       | -15        | +5    | -30        | -45   |
| 0.05                   | 0.2       | -20        | 0     | -35        | -35   |
| 0.01                   | 0.3       | -15        | +10   | -10        | -15   |
| 0.03                   | 0.3       | -15        | -10   | -35        | -45   |
| 0.05                   | 0.3       | -25        | 0     | -40        | -50   |

<sup>1</sup> A 40% concentrate of the acryloid in hydrocarbon solvent.

The data of Table II demonstrate that the microcrystalline wax of the invention is an effective pour depressor aid in acrylate-containing fuels.

**5**  
Example VI

The following tests demonstrate the resistance to solids formation, i.e. suspended (haze) or settled wax precipitates, exhibited by the compositions of the invention using the Mid-Continent microcrystalline wax of the invention, i.e. microcrystalline waxes CFO-1N, CFO-2N, CFO-3N and ECDH of Examples I through IV, in comparison to a Mid-Continent microcrystalline wax having a M.P. of 161° F. (Wax A).

The tests comprised storing samples of a depressed No. 2 fuel, i.e. containing the combination of additives, in 4 oz. bottles under conditions of room temperatures of 40° F. After 48 hours the samples were inspected for visual haze, wax flocculants or wax precipitate. The concentrations of the additives and the results of the tests are shown in Table III.

5

**6**

at room temperature was placed in a 275-gallon fuel storage tank in a cold room, maintained at a constant temperature of either +10° F., -8° F. or 15° F., and the tank was manifolded to a home burner pump located in an adjacent warm room at normal temperatures. Immediately preceding the pump in the warm room was a filter. The test fuel was routed from the pump under a pressure of 100 p.s.i. through a total gallonage meter to a 75 g.p.h. nozzle, thence to discard. The pump was operated on a 20-minutes on, 10-minutes off basis, starting immediately after charging the fuel to the tank. Pumpability failure was taken as the point when fuel ceased to be pumped over a time period of at least 30 minutes, and the percentage of initial fuel oil charge removed from the tank was determined. The results of the tests, the concentration of additives utilized and the

TABLE III.—PRECIPITATE FORMATION IN FUELS CONTAINING MICRO-CRYSTALLINE WAXES  
[Bottle Storage Test at 40° F.]

| Microcrystalline Wax | Inspection After +40° F. Storage 48 Hours |                 |              |             |          |                  |
|----------------------|-------------------------------------------|-----------------|--------------|-------------|----------|------------------|
|                      | Percent Vol.                              | Pour Depressant | Percent Vol. | Visual Haze | Wax Floc | Wax Ppt., Inches |
| Wax A.....           | 0.1                                       | Acryloid 763.   | 0.02         | Yes.....    | No.....  | 1/6              |
|                      | 0.2                                       | do.....         | 0.02         | Yes.....    | No.....  | 1/4              |
|                      | 0.3                                       | do.....         | 0.02         | Yes.....    | No.....  | 1/4              |
|                      | 0.4                                       | do.....         | 0.02         | Yes.....    | No.....  | 1/2              |
| ECDH.....            | 0.1                                       | do.....         | 0.02         | No.....     | No.....  | 0                |
|                      | 0.2                                       | do.....         | 0.02         | No.....     | No.....  | 0                |
|                      | 0.3                                       | do.....         | 0.02         | No.....     | No.....  | 0                |
|                      | 0.4                                       | do.....         | 0.02         | No.....     | No.....  | 0                |
| CFO-1N.....          | 0.1                                       | do.....         | 0.02         | No.....     | No.....  | 0                |
|                      | 0.2                                       | do.....         | 0.02         | No.....     | No.....  | 0                |
|                      | 0.3                                       | do.....         | 0.02         | No.....     | No.....  | 0                |
|                      | 0.4                                       | do.....         | 0.02         | No.....     | No.....  | 0                |
| CFO-2N.....          | 0.1                                       | do.....         | 0.02         | No.....     | No.....  | 0                |
|                      | 0.2                                       | do.....         | 0.02         | No.....     | No.....  | 0                |
|                      | 0.3                                       | do.....         | 0.02         | No.....     | No.....  | 0                |
|                      | 0.4                                       | do.....         | 0.02         | No.....     | No.....  | 0                |
| CFO-3N.....          | 0.1                                       | do.....         | 0.02         | No.....     | No.....  | 0                |
|                      | 0.2                                       | do.....         | 0.02         | No.....     | No.....  | 0                |
|                      | 0.3                                       | do.....         | 0.02         | No.....     | No.....  | 0                |

**Example VII**

No. 2 fuel oil compositions containing small amounts

pour and cloud points of the compositions are shown in Table IV.

TABLE IV.—THE EFFECT OF ADDITIVES ON PUMPABILITY FULL-SCALE TEST

| Additives                    |                    |                | Cloud/<br>Pour | Percent Pumped |        |         |         |
|------------------------------|--------------------|----------------|----------------|----------------|--------|---------|---------|
| Vol. Percent<br>Acryloid 763 | Pour<br>Depressant | Vol. Wax       |                | 0° F.          | -5° F. | -10° F. | -15° F. |
|                              |                    | Fuel Oil A.... | +2/0           | 100            | 83     | 36      | 27      |
| 0.02                         | 0.2 ECDH.....      | do.....        | +5/-5.....     | 100            | .....  | .....   | 86      |
| 0.02                         | 0.2 CFO-1N.....    | do.....        | +8/0.....      | 79             | .....  | .....   | 56      |
| 0.02                         | 0.2 CFO-2N.....    | do.....        | +5/-5.....     | 97             | .....  | .....   | 84      |
| 0.02                         | 0.2 CFO-3N.....    | do.....        | +5/-13.....    | 100            | .....  | .....   | 90      |
| 0.02                         | 0.2 CFO-CN.....    | do.....        | +2/-5.....     | 90             | .....  | .....   | 83      |
| 0.02                         | 0.2 CFO-CB.....    | do.....        | +4/-10.....    | 100            | .....  | .....   | .....   |
| 0.02                         | 0.1 CFO-2.....     | do.....        | +2/0.....      | 100            | .....  | .....   | 82      |
| 0.02                         | 0.2 CFO-2.....     | do.....        | +2/-10.....    | 100            | .....  | .....   | 66      |
| 0.01                         | 0.2 CFO-CN.....    | do.....        | +5/-5.....     | 39             | .....  | .....   | 52      |
| 0.00                         | 0.2 CFO-CN.....    | do.....        | +7/0.....      | 89             | .....  | .....   | 44      |
| 0.02                         | 0.4 CFO-1N.....    | do.....        | +6/-8.....     | 100            | .....  | .....   | 100     |
|                              |                    | Fuel Oil B.... | +4/-5.....     | 92             | .....  | .....   | 43      |
| 0.02                         | 0.2 ECDH.....      | do.....        | +6/-10.....    | 95+            | .....  | .....   | 98      |
| 0.02                         | 0.2 CFO-1N.....    | do.....        | +5/-8.....     | 100            | .....  | .....   | 90      |
| 0.02                         | 0.2 CFO-2N.....    | do.....        | +4/-25.....    | 100            | .....  | .....   | 100     |
| 0.02                         | 0.2 CFO-3N.....    | do.....        | +7/-23.....    | 100            | .....  | .....   | 100     |
| 0.02                         | 0.2 CFO-CN.....    | do.....        | +6/-15.....    | 100            | .....  | .....   | 97      |
| 0.02                         | 0.2 CFO-CB.....    | do.....        | +5/-23.....    | 100            | .....  | .....   | 99      |
| 0.01                         | 0.2 CFO-CN.....    | do.....        | +4/-10.....    | 100            | .....  | .....   | 99      |
| 0.00                         | 0.2 CFO-CN.....    | do.....        | +6/-5.....     | 99             | .....  | .....   | 80      |
| 0.02                         | 0.4 CFO-1N.....    | do.....        | +5/-10.....    | 100            | .....  | .....   | 100     |

of either Acryloid 763, or the microcrystalline waxes identified in Examples I to IV and Table I above and samples containing a combination of the two additives were subjected to a pumpability test over a temperature range of 0 to -15° F. For comparison the neat fuel was also tested. The No. 2 fuels employed are those identified in Example IV above.

The pumpability test employed comprises the following:

40 gallons of the fuel composition tested while still

70 The data of Table IV show that not only is the microcrystalline wax of the invention an excellent pour depressor aid when used in combination with an acrylic acid ester polymer but it is also an excellent pumpability aid over low temperature ranges.

It is claimed:

1. A fuel composition consisting essentially of a petroleum distillate fuel boiling above the gasoline range having incorporated therein about 0.001 to 0.1 volume percent of a viscous, oil-soluble acrylic acid ester poly-

mer pour depressor and about 0.1 to 1 volume percent of a petroleum microcrystalline wax having a melting point of up to about 145° F. and derived from a Mid-Continent base crude oil, said amounts being sufficient to provide said fuel with a reduced pour point and improved pumpability.

2. The composition of claim 1 wherein the melting point of the microcrystalline wax is below about 100° F.

3. The composition of claim 2 wherein the amount of said microcrystalline wax is about 0.2 volume percent up to 0.5 volume percent and the amount of acrylic acid ester polymer pour depressor is about 0.003 to 0.05 volume percent.

## References Cited

## UNITED STATES PATENTS

2,917,375 12/1959 Hudson ----- 44—62

5 DANIEL E. WYMAN, *Primary Examiner.*

Y. H. SMITH, *Assistant Examiner.*

U.S. Cl. X.R.

10 44—70, 80